

May 31, 1932.

H. KLENCKE

1,861,122

PROCESS OF ROASTING AND SINTERING PULVERULENT  
ORES HAVING A HIGH SULPHUR CONTENT

Filed Sept. 16, 1930



Inventor:

Hans Klencke

By Byrnes, Townsend & Potter

his Attorneys.

## UNITED STATES PATENT OFFICE

HANS KLENCKE, OF FRANKFORT-ON-THE-MAIN, GERMANY, ASSIGNOR TO AMERICAN LURGI CORPORATION, OF NEW YORK, N. Y., A CORPORATION OF NEW YORK

PROCESS OF ROASTING AND SINTERING PULVERULENT ORES HAVING A HIGH SULPHUR CONTENT

Application filed September 16, 1930, Serial No. 482,377, and in Germany September 28, 1929.

This invention relates to a process of roasting and sintering pulverulent ores having a high sulphur content.

More particularly the invention relates to a blast roasting or sintering process.

In ore treating processes of the so-called Dwight-Lloyd type, see General Metallurgy by Hoffman, 1913 edition, page 430, the ore to be roasted and sintered is deposited from a feeding-hopper onto pallets which are carried successively under the ore feeding hopper and an igniting furnace and over a suction box. The igniting furnace ordinarily is fired with oil or gas and serves to ignite the ore which then continues to burn in the draft of air passing through it created by the suction box. In accordance with the present invention the igniting furnace is fired with powdered ore of high sulphur content, which is capable of burning whereby not only is the ore on the pallets ignited, but the powdered ore used as fuel in the igniting furnace is roasted and sintered. A burner of the type commonly used for burning powdered coal may be used for feeding the powdered ore to the igniting furnace.

In many cases pulverulent ore alone will not suffice as fuel and it will be necessary to mix it with a certain proportion of other fuels such as for example, gas, coal-dust or the like.

When employing an ore-fired furnace for the ignition, in accordance with the present invention, the burning ore is blown on to the ore layer on the grate which acts as a filter and is roasted and sintered together with said layer.

The fuel which is employed for the ignition furnace in carrying out the invention may comprise pulverulent ores having a high sulphur content such as for example pyrites and zinc blende such as obtained from flotation processes.

The firing with pulverulent ore has the advantage that the firing is utilized for roasting the highly sulphurous ores so that the ores need not, as hitherto usual, be preliminarily roasted and brought into a crumbly form.

The invention will be described further with reference to the accompanying drawing

in which the single figure is a schematic representation of one form of apparatus adapted for the carrying out of the process of the invention.

In the drawing, the numeral 1 indicates the grate of a sintering furnace of the Dwight-Lloyd type. 2 is a feed bunker for laying on the grate 1 a grate-covering charge 6, while 3 is a feed bunker for laying the actual ore charge 7 to be sintered on the protective layer 6. 4 represents an open-bottomed igniting furnace, or combustion chamber, of suitable shape and size and so positioned with respect to the grate and charge of the sintering furnace as to bring its solid and/or gaseous contents into direct contact with the charge 7. 5 diagrammatically represents a suitable nozzle for injecting a combustion-supporting gas-pulverulent ore mixture with or without added fuel into the chamber 4 from any suitable source. 8 indicates the customary suction boxes of apparatus of this type. 9 represents a layer of sintered pulverulent ore superposed on the ore charge layer 7.

The process proceeds as follows: During the passage of the grate 1 below the feed bunkers 2 and 3 a thin layer of protective covering 6 for the grate is applied to the latter, as by shaking, and a layer 7 (of ordinary thickness) of the ore to be sintered is applied thereon. The ignition of this ore layer is accomplished under the chamber or furnace 4. In the latter, a mixture of pulverulent ore of high sulphur content and a gaseous supporter of combustion, e. g., air, with or without an addition of a supplemental fuel, is caused to burn after the manner of ignition customary in the burning of coal dust. The burning pulverulent ore and the resulting gases, actuated by the suction of suction boxes 8, are sucked down onto the charge layer 7 wherein or whereon the solids 9 are retained as on a filter. This burning upper layer serves to ignite the charge layer and is roasted and sintered with the latter.

I claim:—

1. In processes of blast roasting sulphide ores involving depositing a layer of the ore on a grate, igniting the surface of the de-

- posited layer of ore and continuing the sintering of the ore by passing a current of air through the deposited layer, the step which consists in igniting the surface of the deposited layer of ore by burning powdered sulfid ore suspended in a blast of air in contact with said layer of ore whereby said powdered ore is deposited on said layer of ore and roasted and sintered.
- 10 2. Process of blast roasting sulphide ores as defined in claim 1, in which a powdered carbonaceous fuel is mixed with the powdered sulfid ore used for igniting the layer of ore.
- 15 In testimony whereof, I affix my signature.  
HANS KLENCKE.

20

25

30

35

40

45

50

55

60

65